# EUROPEAN PATENT SPECIFICATION

(11) **EP 3 178 911 B1**
(45) Date of publication and mention of the grant of the patent: **30.10.2019**
(21) Application number: 15830586.2
(22) Date of filing: 22.05.2015
(51) Int. Cl.: C10M 169/04, C10M 101/02, C10M 129/10, C10M 133/12, C10M 137/04, C10N 30/06, C10N 30/10, C10N 40/06

(54) **LUBRICATING OIL COMPOSITION**
SCHMIERÖLZUSAMMENSETZUNG
COMPOSITION D'HUILE LUBRIFIANTE

(30) Priority: 06.08.2014 JP 2014160395
(43) Date of publication of application: 14.06.2017
(73) Proprietor: Idemitsu Kosan Co., Ltd, Tokyo 100-8321 (JP)
(72) Inventor: SAKANOUE Shuichi, Ichihara-shi Chiba 299-0107 (JP)
(74) Representative: Vossius & Partner Patentanwälte Rechtsanwälte mbB
(86) International application number: PCT/JP2015/064722
(87) International publication number: WO 2016/021274

(56) References cited:
- EP-A1- 2 067 845
- JP-A- H0 797 586
- JP-A- S6 279 295
- JP-A- 2000 109 873
- JP-A- 2001 003 071
- JP-A- 2007 291 357
- JP-A- 2009 235 268
- JP-A- 2011 068 801
- US-A- 4 634 543
- US-A- 5 536 423

## Description

### TECHNICAL FIELD

The present invention relates to a lubricating oil composition, for instance, to a lubricating oil composition to be used for a shock absorber in an automobile and industrial machinery/device.

### BACKGROUND ART

A shock absorber is provided at a connection portion between tires and a vehicle body in an automobile and is configured to damp vibration of the vehicle body caused by a bumpy road surface and acceleration/deceleration of the automobile. Accordingly, riding comfort on the automobile is considerably affected by a performance of the shock absorber.

Friction of the shock absorber is mainly generated on an oil seal (a rubber material) and a rod (chrome-plated) portion. Accordingly, an improvement in friction characteristics generated between the rubber material and the chrome-plated portion is a very crucial problem. Moreover, in order that the rod of the shock absorber smoothly moves in extension and contraction, an absolute value (a friction coefficient between the rubber material and metal) of rubber friction is required to be small.

The friction characteristics have been so far evaluated in terms of the absolute value of the rubber friction. Accordingly, a shock absorber oil having a small value with respect to the above parameter has been developed (see non-Patent Literatures 1 and 2).

### CITATION LIST

### NON-PATENT LITERATURE(S)

Non-Patent Literature 1: Proceedings of Petroleum Product Symposium of Petroleum Institute, page 96 (December in 2009)
Non-Patent Literature 2: Tribologists, page 567, Vol. 56, No. 9 (in 2011)
Patent Literature 1: US4634543
Patent Literature 2: US5536423

Patent Literature 1 and 2 disclose shock absorber fluids comprising as additive phosphoric acid ester.

### SUMMARY OF THE INVENTION

### PROBLEMS TO BE SOLVED BY THE INVENTION

The absolute values of the rubber friction as described in non-Patent Literatures 1 and 2 are not enough to sufficiently evaluate friction characteristics, so that development of the lubricating oil having excellent friction characteristics has not been easy. Moreover, it has been found that a large workload of the friction (i.e., friction energy) is also crucial for damping vibration of the vehicle body. Further, since the shock absorber is not supposed to be replaced, the shock absorber is generally used continuously for 5 to 10 years. Accordingly, the lubricating oil used for the shock absorber is required to also have a high oxidation stability.

An object of the invention is to provide a lubricating oil composition having a small friction coefficient between a rubber material and metal, a large friction energy and an excellent oxidation stability.

### MEANS FOR SOLVING THE PROBLEM(S)

The invention is defined in the claims. Furthermore, the following is disclosed:
a lubricating oil composition provided by blending to a base oil at least one of acid phosphate represented by formulae (1) and (2) below; and an antioxidant.

In the formulae, R¹, R² and R³ are alkyl groups. At least one of R¹ and R² has 20 to 30 carbon atoms while R³ has 20 to 30 carbon atoms.

According to the above aspect of the invention, a lubricating oil composition having a small friction coefficient between a rubber material and metal, a large friction energy and an excellent oxidation stability can be provided.

### BRIEF DESCRIPTION OF DRAWING(S)

Fig. 1 schematically shows an example of ditetracosyl acid phosphate.
Fig. 2 schematically shows an example of dioctacosyl acid phosphate.
Fig. 3 schematically shows an example of distearyl acid phosphate.
Fig. 4 shows a friction tester used in Examples.
Fig. 5 shows an example of a Lissajous waveform obtained by the friction tester.

### DESCRIPTION OF EMBODIMENT(S)

A lubricating oil composition in an exemplary embodiment of the invention (hereinafter also referred to as "the present composition") is provided by blending a predetermined acid phosphate and an antioxidant to a base oil. The present composition will be described in detail below.

### Base Oil

The base oil used in the present composition is not particularly limited. At least one of a mineral oil and a synthetic oil may be used alone or in combination of two or more. Alternatively, a combination of the mineral oil and the synthetic oil may be used.

When the present composition is used for a shock absorber, it is preferable to use a base oil having a kinematic viscosity at 40 degrees C in a range approximately from 5 mm²/s to 40 mm²/s in order to keep suitable friction characteristics.

Moreover, a pour point of the base oil, which is an index for low-temperature fluidity, is preferably -10 degrees C or less, particularly preferably -15 degrees C or less.

Examples of the mineral oil include a naphthenic mineral oil, a paraffinic mineral oil, and GTL WAX. Specifically, the examples of the mineral oil include a light neutral oil, intermediate neutral oil, heavy neutral oil and bright stock which are obtained by solvent purification or hydrogenation purification.

On the other hand, examples of the synthetic oil include polybutene, a hydride thereof, poly-alpha-olefin (e.g., 1-octene oligomer, 1-decene oligomer), alkylbenzene, polyolester, diacid ester, polyoxyalkyleneglycol, polyoxyalkyleneglycolester, polyoxyalkyleneglycolether, hindered ester and silicone oil.

### Acid Phosphate

Acid phosphate contained in the present composition is represented by formulae (1) and (2) below.

In the formulae, R¹, R² and R³ are alkyl groups. At least one of R¹ and R² has 20 to 30 carbon atoms while R³ has 20 to 30 carbon atoms.

Examples of the alkyl group having 20 to 30 carbon atoms include an eicosyl group, heneicosyl group, docosyl group, tricosyl group, tetracosyl group, pentacosyl group, hexacosyl group, heptacosyl group, octacosyl group, nonacosyl group and triacontyl group.

Examples of the acid phosphate represented by the formulae (1) and (2) include tetracosyl acid phosphate, ditetracosyl acid phosphate, octacosyl acid phosphate, and dioctacosyl acid phosphate when R¹ to R³ are a tetracosyl group or an octacosyl group. For reference, an example of ditetracosyl acid phosphate and an example of dioctacosyl acid phosphate are schematically shown in Figs 1 and 2, respectively.

Since the acid phosphate has an alkyl group having 20 or more carbon atoms, a friction coefficient and a friction energy are effectively improvable. Moreover, the oxidation stability is also improvable in the presence of the above-described acid phosphate.

Further, the number of the carbon atoms of the above-described alkyl group is preferably 30 or less since solubility of the acid phosphate in the base oil can be secured. The number of the carbon atoms of the above-described alkyl group is preferably in a range from 20 to 26, more preferably in a range from 20 to 24.

On the other hand, when the number of the carbon atoms of the alkyl group falls below the lower limit described above, the friction coefficient becomes large, so that the friction energy also cannot be expected to be increased. For instance, in Fig. 3 schematically showing an example of distearyl acid phosphate, since the number of the carbon atoms of the alkyl group is small, the friction coefficient becomes large and the friction energy becomes small.

The alkyl group of the formulae (1) and (2)
has a side chain in order to decrease the friction coefficient and increase the friction energy. Further, since the side chain serves as steric hindrance, the oxidation stability is also improvable. Specifically, at least one of R¹ and R² has a side chain in the formula (1), or, R³ has a side chain in the formula (2). Further, the number of the carbon atoms of the above-described side chain is preferably in a range from 6 to 18. The side chain having 6 or more carbon atoms is preferable in terms of a decrease in the friction coefficient and an increase in the friction energy. Moreover, the side chain having 18 or less carbon atoms is preferable since solubility of the acid phosphate in the base oil becomes favorable.

The acid phosphate of the formula (1) is preferable to the acid phosphate of the formula (2) in terms of the decrease in the friction coefficient, the increase in the friction energy and the oxidation stability.

In the present composition, a content of the above-described acid phosphate blended with the base oil is in a range of 0.01 mass% to 3 mass% of the total amount of the composition, preferably in a range of 0.1 mass% to 2 mass%, further preferably in a range of 0.2 mass% to 1 mass%. The content of the acid phosphate of 0.01 mass% or more is chosen not only in terms of the decrease in the friction coefficient and the increase in the friction energy but also the oxidation stability. Moreover, the content of the acid phosphate of 3 mass% or less is chosen since solubility of the acid phosphate in the base oil can be secured.

### Antioxidant

The present composition further contains an antioxidant. Although the predetermined acid phosphate described above has an effect for improving the oxidation stability, use of the antioxidant in combination with the acid phosphate exhibits an outstanding oxidation stability.

As the antioxidant, at least one of an amine antioxidant, a phenolic antioxidant and a sulfur antioxidant is preferably usable. One of the antioxidant may be used alone or a combination of two or more thereof may be used.

Examples of the amine antioxidant includes: monoalkyldiphenylamine compounds such as monooctyldiphenylamine and monononyldiphenylamine; dialkyldiphenylamine compounds such as 4,4'-dibutyldiphenylamine, 4,4'-dipentyldiphenylamine, 4,4'-dihexyldiphenylamine, 4,4'-diheptyldiphenylamine, 4,4'-dioctyldiphenylamine and 4,4'-dinonyldiphenylamine; polyalkyldiphenylamine compounds such as tetrabutyldiphenylamine, tetrahexyldiphenylamine, tetraoctyldiphenylamine and tetranonyldiphenylamine; and naphthylamine compounds such as α-naphthylamine, phenyl-α-naphthylamine, butylphenyl-α-naphthylamine, pentylphenyl-α-naphthylamine, hexylphenyl-α-naphthylamine, heptylphenyl-α-naphthylamine, octylphenyl-α-naphthylamine and nonylphenyl-α-naphthylamine.

Examples of the phenolic antioxidant include: monophenol compounds such as 2,6-di-tert-butyl-4-methylphenol and 2,6-di-tert-butyl-4-ethylphenol; and diphenol compounds such as 4,4'-methylenebis(2,6-di-tert-butylphenol) and 2,2'-methylenebis(4-ethyl-6-tert-butylphenol).

Examples of the sulfur antioxidant include: thioterpene compounds such as 2,6-di-tert-butyl-4-(4,6-bis(octylthio)-1,3,5-triazine-2-yl amino)phenol and a reactant of phosphorus pentasulfide and pinene; and dialkylthio dipropionates such as dilauryl thiodipropionate and distearyl thiodipropionate.

A content of the antioxidant is from 0.01 mass% to 10 mass% based on the total amount of the composition, preferably approximately from 0.03 mass% to 5 mass%.

In the invention, a "lubricating oil composition provided by blending a predetermined acid phosphate and an antioxidant to a base oil" encompasses not only a "lubricating oil composition containing a base oil, a predetermined acid phosphate and an antioxidant" but also a composition containing a modified substance of at least one of the "base oil," "predetermined acid phosphate" and "antioxidant" in place of the at least one of the "base oil," "predetermined acid phosphate" and "antioxidant" and a composition containing a reaction product obtained by reacting the "base oil," "predetermined acid phosphate" and "antioxidant."

### Other Components

The present composition may be added as needed with other additives such as a viscosity index improver, a pour point depressant, an antiwear agent, a friction modifier, a metal detergent, an ashless dispersant, a rust inhibitor, a metal deactivator and an antifoaming agent as long as advantages of the invention are not hampered. Moreover, the present composition containing the above additives encompasses a composition containing a modified substance of the additives and a composition containing a reaction product obtained by reacting the additives.

Examples of the viscosity index improver include polymethacrylate, dispersed polymethacrylate, olefin copolymer (e.g. ethylene-propylene copolymer), dispersed olefin copolymer and styrene copolymer (e.g. styrene-diene copolymer and styrene-isoprene copolymer). A content of the viscosity index improver is approximately in a range from 0.5 mass% to 15 mass% of the total amount of the present composition in view of the blending effect thereof.

An example of the pour point depressant is polymethacrylate having a mass average molecular weight approximately in a range from 10000 to 150000. A preferable content of the pour point depressant is approximately in a range from 0.01 mass% to 10 mass% of the total amount of the present composition.

Examples of the antiwear agent include: a sulfur antiwear agent such as a thiophosphoric acid metal salt (e.g., Zn, Pb and Sb) and a thiocarbamic acid metal salt (e.g., Zn); and a phosphorus antiwear agent such as a phosphate (tricresyl phosphate). A preferable content of the antiwear agent is approximately in a range from 0.05 mass% to 5 mass% of the total amount of the present composition.

Examples of the friction modifier include a polyhydric alcohol partial ester such as neopentyl glycol monolaurate, trimethyrol propanemonolaurate, and glycerin monooleate (oleic acid monoglyceride). A preferable content of the friction modifier is approximately in a range from 0.05 mass% to 4 mass% of the total amount of the present composition.

The metal detergent is preferably at least one of metal salicylate, metal phenate and metal sulfonate. The metal is preferably alkaline earth metal, more preferably Ca. Ca salicylate is particularly preferable in order to retain the detergency. A base value of the metal detergent according to a hydrochloric acid method is preferably in a range from 100 mgKOH/g to 250 mgKOH/g in order to retain the detergency. A content of the metal detergent is preferably in a range from 60 mass ppm to 6000 mass ppm based on the total amount of the composition and in terms of the metal amount.

Examples of the ashless dispersant include succinimides, boron-containing succinimides, benzylamines, boron-containing benzylamines, succinic acid esters, and mono- or di-carboxylic acid amides respectively represented by a fatty acid or succinic acid. A preferable content of the ashless dispersant is approximately in a range from 0.1 mass% to 20 mass% of the total amount of the present composition.

Examples of the rust inhibitor include a fatty acid, alkenylsuccinic acid half ester, fatty acid soap, alkyl sulfonate, fatty acid ester of polyhydric alcohol, fatty acid amide, oxidized paraffin and alkyl polyoxyethylene ether. A preferable content of the rust inhibitor is approximately in a range from 0.01 mass% to 3 mass% of the total amount of the present composition.

One of the metal deactivators such as benzotriazole and thiadiazole may be used alone, or a combination of two or more thereof may be used. A preferable content of the metal deactivator is approximately in a range from 0.01 mass% to 5 mass% of the total amount of the present composition.

One of the antifoaming agents such as a silicone compound and an ester compound may be used alone, or a combination of two or more thereof may be used. A preferable content of the antiwear agent is approximately in a range from 0.05 mass% to 5 mass% of the total amount of the present composition.

Since the present composition contains the acid phosphate having a predetermined structure and the antioxidant, the friction coefficient between the rubber material and the metal is small, the friction energy is large, and the oxidation stability is excellent. Accordingly, the present composition is suitably usable for the shock absorber, particularly suitably usable for the shock absorber of a four-wheel automobile (e.g., a passenger car, bus and truck) in which riding comfort is of great interest.

Moreover, the present composition is also suitably usable for a shock absorber of a two-wheel vehicle. Further, the present composition is suitably usable as hydraulic fluid. Examples

The invention will be further described in detail below by reference to Examples and Comparatives, which by no means limit the invention. Properties and performance of the lubricating oil composition (sample oil) in each of Examples and Comparatives were obtained in accordance with the following methods.

### (1) Kinematic Viscosity at 40 Degrees C

A kinematic viscosity at 40 degrees C of the present composition was measured in accordance with JIS K 2283.

### (2) Increase Ratio of Kinematic Viscosity at 40 Degrees C

After the present composition was subjected to an ISOT test (in accordance with JIS K 2514: 130°C, 24 hours), a kinematic viscosity at 40 degrees C of the present composition was measured. An increase ratio in the kinematic viscosity at 40 degrees C of the present composition after the ISOT test relative to the present composition before the ISOT test was obtained.

### (3) Friction Coefficient and Friction Energy

The friction coefficient (kinematic friction coefficient) between the rubber and the metal and the friction energy were obtained using a tester shown in Fig. 4. Specifically, as shown in Fig. 4, rubber and a Cr (chrome)-plated steel plate were reciprocatingly slid while being in pressure contact with each other at a predetermined load through a sample oil, and a Lissajous waveform was recorded. Fig. 5 shows an example of the Lissajous waveform. A friction coefficient (µ) was obtained from the maximum value of a friction force. An area (which is a product of an amplitude and the friction force and corresponds to workload) of the Lissajous waveform was obtained as the friction energy.

Test conditions are shown below.
Temperature: 30 degrees C
Amplitude: ±0.4 mm (sine wave)
Load: 3 kgf (29.4N)
Upper test piece: NBR (nitrile rubber)
Lower test piece: hard Cr-plated steel plate
Excitation Frequency: 5Hz
Sample oil amount: 100 mL

### Examples 1 to 2, Comparatives 1 to 12

Lubricating oil compositions were prepared according to blending compositions shown in Tables 1 and 2. Properties and performance of each of the sample oils were evaluated in accordance with the above-described methods. The results are also shown in Tables 1 and 2.

### Evaluation Results

As understood from Examples 1 and 2, in the sample oils containing a predetermined acid phosphate and the antioxidant, the friction coefficient between the rubber material and the metal is small, the friction energy is large, and the oxidation stability is excellent. According to the invention, it is understandable that a shock absorber oil providing an excellent riding comfort and usable for a long period of time can be provided.

In contrast, the sample oils of Comparatives, in which various agents such as an oiliness agent and a phosphorus extreme pressure agent are blended, cannot simultaneously satisfy all of the friction coefficient, the friction energy and the oxidation stability. For instance, the sample oils in Comparatives 2, 3, 5 and 10 exhibit poor oxidation stability in spite of containing the same amount of the same antioxidant as in Examples 1 and 2. In Comparative 12, the sample oil contains acid phosphate diester having an alkyl group with a relatively large number of carbon atoms. Since the number of the carbon atoms of the alkyl group is 18, which is smaller than the lower limit of the number of the carbon atoms of the alkyl group in the invention, the friction coefficient is large and an increase in the friction energy is hardly recognized as compared with the sample oil with only the base oil (i.e., Comparative 1 only containing the antioxidant).

## Claims

1. A lubricating oil composition comprising:
a base oil;
at least one of acid phosphate represented by formulae (1) and (2) below, wherein the acid phosphate is contained in a range from 0.01 mass% to 3 mass% of a total amount of the composition; and
an antioxidant, wherein the antioxidant is contained in a range from 0.01 mass% to 10 mass%, based on the total amount of the composition,
where: R¹, R² and R³ are alkyl groups; and at least one of R¹ and R² has 20 to 30 carbon atoms while R³ has 20 to 30 carbon atoms, wherein
at least one of R¹ and R² has a side chain, or
R³ has a side chain.

2. The lubricating oil composition according to claim 1, wherein
the side chain has 6 to 18 carbon atoms.

3. The lubricating oil composition according to claim 1 or 2, wherein
the antioxidant is at least one of a phenolic antioxidant, an amine antioxidant and a sulfur antioxidant.

4. Use of the lubricating oil composition according to any one of claims 1 to 3 in a shock absorber.

5. Use according to claim 4 wherein the shock absorber is suitable for use in a four-wheel automobile.

## Patentansprüche

1. Eine Schmierölzusammensetzung, umfassend:
ein Grundöl;
mindestens eines aus einem Säurephosphat dargestellt durch die nachstehenden Formeln (1) und (2), wobei das Säurephosphat in einem Bereich von 0,01 Massen-% bis 3 Massen-% einer Gesamtmenge der Zusammensetzung enthalten ist; und
ein Antioxidans, wobei das Antioxidans in einem Bereich von 0,01 Massen-% bis 10 Massen-%, bezogen auf die Gesamtmenge der Zusammensetzung, enthalten ist,
wobei: R¹, R² und R³ Alkylgruppen sind; und mindestens eines von R¹ und R² 20 bis 30 Kohlenstoffatome aufweist, während R³ 20 bis 30 Kohlenstoffatome aufweist, wobei mindestens eines von R¹ und R² eine Seitenkette aufweist, oder
R³ eine Seitenkette aufweist.

2. Die Schmierölzusammensetzung gemäß Anspruch 1, wobei
die Seitenkette 6 bis 18 Kohlenstoffatome aufweist.

3. Die Schmierölzusammensetzung gemäß Anspruch 1 oder 2, wobei
das Antioxidans mindestens eines aus einem phenolischen Antioxidans, einem Amin-Antioxidans und einem Schwefel-Antioxidans ist.

4. Verwendung der Schmierölzusammensetzung gemäß einem der Ansprüche 1 bis 3 in einem Stoßdämpfer.

5. Verwendung gemäß Anspruch 4, wobei der Stoßdämpfer zur Verwendung in einem vierrädrigen Kraftfahrzeug geeignet ist.

## Revendications

1. Composition d'huile lubrifiante comprenant :
une huile de base ; et
au moins l'un d'un phosphate acide représenté par les formules (1) et (2) ci-dessous, où le phosphate acide est contenu dans une plage de 0,01 à 3 % en poids d'une quantité totale de la composition ; et
un antioxydant, où l'antioxydant est contenu dans une plage de 0,01 à 10 % en poids, sur la base de la quantité totale de la composition,
où : R¹, R² et R³ sont des groupes alkyle ; et au moins un des R¹ et R² a 20 à 30 atomes de carbone tandis que R³ a 20 à 30 atomes de carbone, dans laquelle au moins un des R¹ et R² a une chaîne latérale, ou
R³ a une chaîne latérale.

2. Composition d'huile lubrifiante selon la revendication 1, dans laquelle la chaîne latérale a 6 à 18 atomes de carbone.

3. Composition d'huile lubrifiante selon la revendication 1 ou 2, dans laquelle l'antioxydant est au moins l'un d'un antioxydant phénolique, un antioxydant aminé et un antioxydant soufré.

4. Utilisation de la composition d'huile lubrifiante selon l'une quelconque des revendications 1 à 3 dans un amortisseur.

5. Utilisation selon la revendication 4 dans laquelle l'amortisseur est adapté pour une utilisation dans une voiture à quatre roues.
